

## UNITED STATES PATENT OFFICE.

JAMES W. GRIMES, OF SPRINGFIELD, OHIO, ASSIGNOR OF ONE-HALF TO CHARLES D. RAWSON, OF DES MOINES, IOWA.

## FIREPROOF AND WOOD-PRESERVING PAINT.

1,113,782.

Specification of Letters Patent.

Patented Oct. 13, 1914.

No Drawing.

Application filed February 24, 1913. Serial No. 751,148.

*To all whom it may concern:*

Be it known that I, JAMES W. GRIMES, a citizen of the United States, residing at Springfield, in the county of Clark and State of Ohio, have invented a certain new and useful Fireproof and Wood-Preserving Paint, of which the following is a specification.

The object of my invention is to provide an improved chemical product consisting of mixed subsulfids of copper and lead and tar residue that will have, when heated to a certain degree, the consistency of ordinary paint, and that may be applied with a brush to wood for the purpose of making it fire proof and for preserving it; and my object is further to provide a paint of this kind composed of simple and inexpensive ingredients readily obtainable in any locality, and a treatment or process for said ingredients which may be readily and easily carried on, whereby the resultant product is obtained.

My invention consists in the combination of certain chemical substances, whereby the objects contemplated are attained, as hereinafter more fully set forth, and pointed out in my claims.

My improved paint comprises mixed sulfids of copper, mixed sulfids of lead, and tar residue. The exact proportions of said various elements have not yet been fully determined by me. The result of an analysis made by a skilled chemist of my improved paint is as follows:

|                                                                        |         |
|------------------------------------------------------------------------|---------|
| Free or uncombined sulfur                                              | 1.10%   |
| Lead oxid, PbO, (unchanged)                                            | 1.26    |
| Copper sulfate                                                         | None    |
| Mixed sulfids of copper, computed as cuprous sulfid, Cu <sub>2</sub> S | 1.48    |
| Mixed sulfids of lead, computed as PbS                                 | 4.76    |
| Sulfur dioxide, evolved in process of manufacture                      | 2.10    |
| Carbon disulfid, evolved in manufacture                                | 1.05    |
| Water, evolved in process of manufacture                               | 1.92    |
| Tar, residue                                                           | 86.30   |
|                                                                        | 100.00% |

However, the production of this improved paint can be readily and easily practised by persons skilled in the art as follows: I first provide three pounds of sulfur sublimate, three pounds of powdered lead oxid, two

pounds of powdered copper sulfate, and four gallons of coal tar, which ingredients are treated as follows: They are placed in a vessel which should be at least twice as large in capacity as the bulk of the ingredients when first placed therein. Then heat is applied to the vessel and the compound is boiled. During the boiling the mass is stirred. After being boiled for a short period, the mass will greatly increase in size and during this time while boiling the mass will assume a reddish brown color. During the period while this mass is of a reddish brown color, it is highly inflammable and care should be taken that it does not overflow on the fire and that the gases arising from it do not come in contact with the flame. Shortly after the mass has assumed the reddish brown appearance, it will begin to decrease in quantity in the vessel and will assume a black appearance. After the mass has fallen to about its original size and has assumed the black appearance, it will be heat-resisting and cannot be burned under ordinary conditions. In this condition it is ready for use and when applied to wood surfaces or combustible material will protect the wood from burning. The material should be applied to wood or other surfaces while hot and after it has been heated and cooled, it may be repeatedly reheated.

I claim as my invention:

1. An improved fire proof and preservative paint, comprising mixed sulfids of copper, mixed sulfids of lead, and tar residue.

2. An improved fire proof and preservative paint, comprising mixed sulfids of copper, mixed sulfids of lead, and tar residue formed by boiling sulfur sublimate, lead oxid, copper sulfate, and coal tar in about the proportions stated, and in the manner described.

Springfield, Ohio, Feb. 13, 1913.

JAMES W. GRIMES.

Witnesses:

A. C. LINK,

HELEN M. RUNYAN.